

# UNITED STATES PATENT OFFICE.

KURT RÖMMLER, OF SPREMBERG, GERMANY.

## MANUFACTURE OF ARTIFICIAL CLOTH.

No Drawing. Application filed November 13, 1924, Serial No. 749,645, and in Germany November 19, 1923.

This invention relates to the manufacture of artificial cloth by pasting dust of textile fibres upon a fabric.

Up to this day this kind of cloth has generally been manufactured by the following process. The fabric f. ex. a fine cotton fabric is first impregnated with a paste containing certain filling materials and then dried. Thereafter this pasted fabric is polished and glazed by passing it through a polishing and glazing machine and then provided with a film of sticking and fast drying oil. The dust of textile fibres is scattered immediately upon the cloth prepared this way and after a second drying the process is finished. For the double coating and drying as well as for the necessary polishing and glazing after the first impregnation, which has to be done for the purpose of preventing the adhering oilfilm from blotting, this process is comparatively expensive, requires a long time and the resulting product is comparatively brittle and hard. These disadvantages prevent this kind of cloth from being used for many cases f. ex. for the manufacture and adornment of clothes and hats.

According to this invention the fabric is provided with a thin and equal layer of partly saponified linseed-oil varnish or its substitutes, as f. ex. saponifiable natural or synthetic resins or resin oils, and upon this layer the dust of textile fibres is immediately scattered. This partial saponification specially saponifies the lighter parts of the material and prevents without a preceding impregnation the blotting of the fabric. This composition obtained by partial saponifica-

tion can be spread in a very thin layer upon the fabric without losing its capacity of sticking and by this far cheaper and simpler process a very compact, soft and durable textile, fibre cloth is obtained. The duration of the manufacturing process is shorter and the obtained product can replace velvet without any trouble.

The amount of alcali or caustic alcali, necessary for the partial saponification of the oils or varnishes, depends upon their content of three acids. As a rule the saponification is carried so far, that an emulsion results, which is readily spreadable and does not stick any more, when the process is finished.

*Example.*—99 lbs. of linseed-oil, thickened by cooking, as it is commercially sold as technical merchandise, is mixed at about 68° F. with a solution of 0,441 lb. of crystal soda in 1,65 lbs. of water, until a uniform emulsion is obtained.

I claim:

1. A method of manufacturing artificial cloth consisting in coating a fabric with a composition of a partly saponified oil varnish thickened by cooking, and subsequently sprinkling upon this a coating dust of textile fibres.

2. A method of manufacturing artificial cloth consisting in coating a fabric with a composition of a partly saponified linseed-oil varnish thickened by cooking, and subsequently sprinkling upon this a coating dust of textile fibres.

In testimony whereof I have signed my name to this specification.

KURT RÖMMLER.